# EUROPEAN PATENT SPECIFICATION

(11) **EP 2 806 047 B1**
(45) Date of publication and mention of the grant of the patent: **03.02.2016**
(21) Application number: 14169160.0
(22) Date of filing: 20.05.2014
(51) Int. Cl.: C22C 38/42, C22C 38/44, C22C 38/02, C22C 38/04, C22C 38/06, C22C 38/46, C22C 38/48, C22C 38/50, C22C 38/54, C22C 19/05, C22C 30/00, C22C 30/02, C21D 6/00, C21D 6/02, C22F 1/10, C21D 1/18

(54) **PRECIPITATION HARDENED FE-NI ALLOY**
AUSSCHEIDUNGSGEHÄRTETE FE-NI-LEGIERUNG
ALLIAGE FE-NI DURCI PAR PRÉCIPITATION

(30) Priority: 21.05.2013 JP 2013106957; 28.02.2014 JP 2014039222
(43) Date of publication of application: 26.11.2014
(73) Proprietor: Daido Steel Co.,Ltd., Nagoya Aichi 461-8581 (JP)
(72) Inventor: Takahashi, Mari, Nagoya-shi, Aichi 457-8545 (JP); Ueta, Shigeki, Nagoya-shi, Aichi 457-8545 (JP)
(74) Representative: Diehl & Partner GbR

(56) References cited:
- EP-A1- 0 244 520
- EP-A2- 0 639 654
- WO-A1-2009/060900
- GB-A- 999 439
- GB-A- 1 343 184
- GB-A- 1 372 605
- JP-A- H0 397 823
- JP-A- H0 711 376
- JP-A- H11 117 019
- US-A1- 2009 081 073

## Description

### FIELD OF THE INVENTION

The present invention relates to a precipitation hardened Fe-Ni alloy. More specifically, the invention relates to a precipitation hardened Fe-Ni alloy having high strength and excellent corrosion resistance.

### BACKGROUND OF THE INVENTION

A precipitation hardened stainless steel is a steel in which elements such as Cu, Al, Ti, Nb, and Mo are added to achieve precipitation hardening and has both of high corrosion resistance and high strength. Particularly, an austenite precipitation hardened stainless steel represented by A286 alloy (SUH660) is an alloy excellent in both of corrosion resistance and strength among Fe based alloys. However, for using the austenite precipitation hardened stainless steel as a member requiring high strength in marine environment, it is insufficient in both of corrosion resistance and strength.

On the other hand, in Fe-Ni alloys, alloys to which Ti, Al, and Nb are added have been hitherto proposed.

For example, Patent Document 1 (Example 1) discloses a nickel-iron based alloy comprising, in terms of% by weight, 0.027% of C, 0.08% of Mn, 0.10% of Si, 0.001 % of P, 0.005% of S, 15.81 % of Cr, 39.89% of Ni, 2.83% ofNb, 1.61% of Ti, 0.3% of Al, and 0.0041% of B, with the balance being Fe and unavoidable impurities.

Patent Document 2 (No. 1) discloses an Ni based alloy comprising, in terms of % by weight, 0.017% of C, 0.15% of Si, 0.14% of Mn, 0.010% of P, 0.003% of S, 40.32% of Ni, 16.20% of Cr, 1.02% of Mo, 0.25% of Al, 0.95% of Ti, and 2.71% of Nb, with the balance being Fe and unavoidable impurities.

The document describes a fact that the alloy has high strength from room temperature till extremely low temperature and can suppress HAZ cracking by such a composition.

Furthermore, Patent Document 3 (alloy #7) discloses a high-strength corrosion-resistant alloy comprising, in terms of % by weight, 44.2% of Ni, 19.5% of Cr, 3.4% of Mo, 2.0% of Cu, 0.006% of C, 0.3% of Al, 3.8% ofNb, and 1.6% of Ti, with the balance being Fe.

The document describes a fact that high strength is obtained by precipitating predetermined amounts of the y' phase and the y" phase by annealing and aging treatments.

In Patent Document 1, Mo and Cu are not added and corrosion resistance is insufficient. In Patent Document 2, strength is insufficient owing to the balance among Ni, Nb, Ti, and Al. In Patent Document 3, strength of Ni and Nb are high and the raw material costs and the production costs thereof are high.

Patent Document 4 discloses an austenitic stainless steel product for polymer electrolyte fuel cell separators in which one or more kinds of conductive precipitates having Ni contents of 50 mass% or above are exposed on the surface and the surface-exposure ratio of the precipitates is 3% by area. It is preferable that the precipitates contain Ni3X (wherein X is one or more selected from the group consisting of Al, Ti, V, Nb, Ta and Zr), particularly, Ni3Nb phase and/or Ni3Ti phase.

[Patent Document 1] JP-A-47-042414
[Patent Document 2] JP-A-03-097823
[Patent Document 3] JP-T-2009-515053 (the term "JP-T" as used herein
[Patent Document 4] WO2009/060900 A1 means a published Japanese translation of a PCT patent application)

### SUMMARY OF THE INVENTION

A problem to be solved by the present invention is to provide a precipitation hardened Fe-Ni alloy having both of high corrosion resistance and high hardness.

In order to solve the above problem, the gist of the invention is that the precipitation hardened Fe-Ni alloy according to the invention has the following constitutions.

the precipitation hardened Fe-Ni alloy consisting of:
from 0.01 to 0.08% by mass of C,
from 0.02 to 1.0% by mass of Si,
not more than 1.0% by mass of Mn,
from 36.0 to 41.0% by mass of Ni,
14.0 or more and less than 20.0% by mass of Cr,
from 0.01 to 3.0% by mass of Mo,
from 0.1 to 1.0% by mass of Al,
from 1.0 to 2.5% by mass of Ti, and
from 2.0 to 3.5% by mass of Nb,
from 0.0005 to 0.01% by mass of B,
with the balance being Fe and unavoidable impurities; the precipitation hardened Fe-Ni alloy satisfying the following formulae (1) and (2): optionally comprising:
   0.05 to 1.0% by mass of Cu,
   0.05 to 1.0% by mass of V,
   0.001 to 0.50% by mass of Zr, Ta, W, Hf, Mg and REM in total, and from 0.0005 to 0.01% by mass of Ca, $Ni \geq 6 \times Nb + 17$ $Nb / \left(Ti+Al\right) \geq 0.8$

It is preferred that the precipitation hardened Fe-Ni alloy satisfies the following formula (3): $Cr + 3 ⁢ Mo + 5 ⁢ Cu \geq 19$

When predetermined amounts of Nb, Al, and Ti are added to a precipitation hardened Fe-Ni alloy, the y' phase (Ni₃(Al, Ti, Nb)) and the y" phase (Ni₃Nb) containing Nb as a constituent element are precipitated by a solution heat treatment and an aging treatment.

At this time, when the Nb content is optimized so as to satisfy the formula (2), the precipitation amount of the y" phase is increased. Therefore, high strength can be obtained as compared with the conventional alloys.

On the other hand, as the addition amount of Nb increases, the Laves phase (Fe₂Nb) is prone to remain after the solution heat treatment. When the Laves phase remains in a large amount, the Nb amount necessary for precipitation hardening in the matrix decreases. As a result, necessary hardness cannot be obtained even when the aging treatment is performed.

Contrarily, when the Ni content is optimized so as to satisfy the formula (1), the remaining of the Laves phase can be suppressed after the solution heat treatment.

Furthermore, when predetermined amounts of Cr and Mo are added to the precipitation hardened Fe-Ni alloy or predetermined amounts of Cr, Mo and Cu are added to the precipitation hardened Fe-Ni alloy, high corrosion resistance is obtained with maintaining high strength. Particularly, when the contents of Cr, Mo and Cu are optimized so as to satisfy the formula (3), high corrosion resistance is obtained.

### BRIEF DESCRIPTION OF THE DRAWINGS

Fig. 1 shows optical microscopic pictures of the materials after a solution heat treatment obtained in Example 5 and Comparative Example 4.

### DETAILED DESCRIPTION OF THE INVENTION

The following will describe one embodiment of the invention in detail.

### [1: Precipitation Hardened Fe-Ni Alloy]

### [1.1. Main Constituent Elements]

The precipitation hardened Fe-Ni alloy according to the invention contains the following elements, with the balance being Fe and unavoidable impurities. Kinds of the addition elements, composition ranges thereof, and reasons for the limitation thereof are as follows.

### (1) C: from 0.01 to 0.08% by mass

C is an element effective for forming a carbide together with Nb and Ti to enhance the strength. Moreover, it suppresses crystal grain coarsening at a solution heat treatment. For obtaining such effects, the C content is necessarily 0.01% by mass or more. The C content is further preferably 0.04% by mass or more.

On the other hand, when the C content becomes excessive, toughness and ductility are lowered. Moreover, when a large amount of the carbide is formed, corrosion resistance is remarkably lowered. For suppressing the lowering of the toughness and ductility and the corrosion resistance, the C content is necessarily 0.08% by mass or less. The C content is preferably 0.07% by mass or less.

### (2) Si: from 0.02 to 1.0% by mass

Si is effective as a deoxidizing element at the time of ingoting. For obtaining such an effect, the Si content is necessarily 0.02% by mass or more.

On the other hand, when the Si content becomes excessive, the toughness is lowered. Therefore, the Si content is necessarily 1.0% by mass or less.

### (3) Mn: not more than 1.0% by mass

Similarly to Si, Mn is effective as a deoxidizing element at the time of ingoting. However, when a large amount thereof is added, oxidation resistance at a high temperature is lowered. Moreover, excessive Mn also lowers corrosion resistance. Therefore, the Mn content is necessarily 1.0% by mass or less.

### (4) Ni: from 36.0 to 41.0% by mass

Ni is essential as an austenite-forming element. Also, Ni makes the alloy age-hardened through precipitation of the y' phase (Ni₃(Al, Ti, Nb)) and the y" phase (Ni₃Nb) together with Ti, Al, and Nb by the aging treatment. For obtaining such an effect, the Ni content is necessarily 36.0% by mass or more. The Ni content is more preferably 37.0% by mass or more.

On the other hand, when the Ni content becomes excessive, the raw material costs are increased. Therefore, the Ni content is necessarily 41.0% by mass or less. The Ni content is more preferably 40.0% by mass or less, further preferably 39.0% by mass or less.

### (5) Cr: 14.0 or more and less than 20.0% by mass

Cr is an inevitable component for enhancing the corrosion resistance of the precipitation hardened Fe-Ni alloy. For obtaining such an effect, the Cr content is necessarily 14.0% by mass or more.

However, Cr is a ferrite-forming element and, when the Cr content becomes excessive, structural stability is lowered. Also, excessive Cr lowers hot workability. Therefore, the Cr content is necessarily less than 20.0% by mass. The Cr content is more preferably 18.0% by mass or less, further preferably 17.0% by mass or less.

### (6) Mo: from 0.01 to 3.0% by mass

Mo improves the corrosion resistance (particularly pitting resistance) through solution into the parent phase. For obtaining such an effect, the Mo content is necessarily 0.01 % by mass or more.

On the other hand, when the Mo content becomes excessive, the Laves phase (Fe₂(Mo, Nb)) is precipitated at the time of the aging treatment and the precipitation amounts of the y' phase and the y" phase are decreased. As a result, the strength of the alloy is lowered. Therefore, the Mo content is necessarily 3.0% by mass or less. The Mo content is preferably 2.0% by mass or less.

### (7) Al: from 0.1 to 1.0% by mass

Al makes the alloy age-hardened through precipitation of the y' phase (Ni₃(Al, Ti, Nb)) together with Ni, Ti, and Nb. For obtaining such an effect, the Al content is necessarily 0.1% by mass or more.

When the Al content becomes excessive, the hot workability is lowered. Therefore, the Al content is necessarily 1.0% by mass or less. The Al content is preferably 0.5% by mass or less.

### (8) Ti: from 1.0 to 2.5% by mass

Ti makes the alloy age-hardened through precipitation of the γ' phase (Ni₃(Al, Ti, Nb)) together with Ni, Al, and Nb. For obtaining such an effect, the Ti content is necessarily 1.0% by mass or more. The Ti content is preferably 1.5% by mass or more, more preferably 1.8% by mass or more.

On the other hand, when the Ti content becomes excessive, the hot workability is lowered. Therefore, the Ti content is necessarily 2.5% by mass or less.

### (9) Nb: from 2.0 to 3.5% by mass

Nb makes the alloy age-hardened through precipitation of the γ' phase (Ni₃(Al, Ti, Nb)) and the y" phase (Ni₃Nb) together with Ni. For obtaining such an effect, the Nb content is necessarily 2.0% by mass or more.

On the other hand, when the Nb content becomes excessive, a coarse Laves phase remains after the solution heat treatment and the precipitation amounts of the y' phase and the y" phase are decreased. As a result, required strength and hardness are not obtained. Therefore, the Nb content is necessarily 3.5% by mass or less. The Nb content is more preferably 3.0% by mass or less.

### [1.2. Auxiliary Constituent Elements]

The precipitation hardened Fe-Ni alloy according to the invention may further contain one kind or two or more kinds of the following auxiliary constituent elements in addition to the aforementioned main constituent elements. Kinds of the addition elements, composition ranges thereof, and reasons for the limitation thereof are as follows.

### (10) B: from 0.0005 to 0.01% by mass

B has an effect of enhancing the hot workability by adding B in a small amount. Also, the precipitation of the η phase at a grain boundary can be suppressed by the presence of B at the grain boundary. For obtaining such an effect, the B content is 0.0005% by mass or more. The B content is preferably 0.0010% by mass or more. The B content is particularly preferably 0.0020% by mass or more.

On the other hand, when the B content becomes excessive, the hot workability is lowered. Therefore, the B content is 0.01% by mass or less. The B content is preferably 0.008% by mass or less.

### (11) Cu: from 0.05 to 1.0% by mass

Cu has an effect of enhancing the corrosion resistance in a non-oxidative corrosive environment. For obtaining such an effect, the Cu content is 0.05% by mass or more. The Cu content is preferably 0.10% by mass or more.

On the other hand, when the Cu content becomes excessive, the hot workability is lowered. Therefore, the Cu content is 1.0% by mass or less.

### (12) V: from 0.05 to 1.0% by mass

As is the case with Nb and Ti, V forms a carbide to enhance the strength. Also, the precipitation amounts of the γ' phase and the y" phase are increased through reducing the ratio of Nb in the carbide. For obtaining such effects, the V content is 0.05% by mass or more.

On the other hand, when the V content becomes excessive, the toughness and the processability are lowered. Therefore, the V content is 1.0% by mass or less.

### (13) Zr, Ta, W, Hf, Mg, and/or REM: from 0.001 to 0.50% by mass in total

Zr, Ta, W, Hf, Mg, and REM (Rare Earth Metal) have an effect on micronization of the carbide and micronization of crystal grains. For obtaining such an effect, a total content of these elements is 0.001% by mass or more.

On the other hand, when the content of these elements becomes excessive, the toughness is lowered. Therefore, the total content of these elements is 0.50% by mass or less.

Incidentally, any one of these elements may be added or two or more thereof may be used in combination.

### (14) Ca: from 0.0005 to 0.01% by mass

Ca improves machinability. For obtaining such an effect, the Ca content is 0.0005% by mass or more.

On the other hand, when the Ca content becomes excessive, the hot workability is lowered. Therefore, the Ca content is 0.01% by mass or less.

### [1.3. Component Balance]

The precipitation hardened stainless steel according to the invention necessarily satisfies the following formulae (1) and (2), in addition to the requirement that the constituent elements are present in the aforementioned ranges.

Moreover, for obtaining high corrosion resistance, the precipitation hardened stainless steel preferably further satisfies the following formula (3). $Ni \geq 6 \times Nb + 17$ $Nb / \left(Ti+Al\right) \geq 0.8$ $Cr + 3 ⁢ Mo + 5 ⁢ Cu \geq 19$

### [1.3.1. Formula (1)]

The formula (1) is relevant to the amount of the Laves phase after the solution heat treatment. When the Ni amount and the Nb amount are optimized so as to satisfy the formula (1), the Laves phase (Fe₂Nb) can be completely dissolved after the solution heat treatment. As a result, the precipitation amounts of the γ' phase and the y" phase at the time of the aging treatment are increased and thereby the strength of the alloy is enhanced.

The formula (1) is more preferably Ni≥6×Nb+18.0, further preferably Ni≥6×Nb+20.0.

### [1.3.2. Formula (2)]

The formula (2) is relevant to the amount of the y" phase at the time of the aging treatment. When the amounts of Nb, Ti, and Al are optimized so as to satisfy the formula (2), the precipitation amount of the y" phase is increased and thereby further enhancing the strength of the alloy.

### [1.3.3. Formula (3)]

The formula (3) is relevant to the corrosion resistance of the precipitation hardened Fe-Ni alloy. Cr, Mo, and Cu all have an effect of enhancing the corrosion resistance of the precipitation hardened Fe-Ni alloy. Particularly, when the contents of these elements are optimized so as to satisfy the formula (3), high corrosion resistance is exhibited with maintaining high strength.

### [1.4.0.2% Offset Yield Strength]

When individual components are optimized as mentioned above and a suitable solution heat treatment is performed, the Laves phase is almost completely dissolved in the matrix. When such a material is subjected to a suitable aging treatment, large amounts of the y' phase and the y" phase are precipitated. As a result, the 0.2% offset yield strength at room temperature becomes 850 MPa or more. When the components and the heat treatment conditions are further optimized, the 0.2% offset yield strength at room temperature becomes 900 MPa or more or 950 MPa or more.

### [1.5. Area Percentage of Carbide]

The precipitation hardened Fe-Ni alloy according to the invention is preferably one in which an area percentage of the carbide after the solution heat treatment is 0.4% or more. At the time of the solution heat treatment, the coarsening of crystal grains can be suppressed when a predetermined amount of the carbide is dispersed in the matrix.

Here, the "area percentage of the carbide" means a ratio of area of the carbide to the total area of cross-sectional microstructure (0.034 mm² × 30 viewing fields).

### [2. Method for Manufacturing Precipitation Hardened Fe-Ni Alloy]

The method for manufacturing the precipitation hardened Fe-Ni alloy according to the invention comprises a melting and casting process, a hot working process, a solution heat treatment process, and an aging treatment process.

### [2.1. Melting and Casting Process]

The melting and casting process is a process of dissolving a raw material blended in a predetermined composition and performing casting. The dissolving method and the casting method are not particularly limited and various methods can be used according to the purpose.

### [2.2. Hot Working Process]

The hot working process is a process of hot-working an ingot obtained in the melting and casting process. The hot working is performed for destroying cast structure and casting defect. Hot working conditions are not particularly limited and most suitable conditions can be selected according to the purpose.

### [2.3. Solution Heat Treatment Process]

The solution heat treatment process is a process of heating a hot-worked material at a predetermined temperature.

The solution heat treatment is performed mainly for dissolving a precipitate dispersed in the steel. When heat treatment temperature is too low, solution of the precipitate becomes insufficient. The heat treatment temperature is preferably 900°C or higher.

On the other hand, when the heat treatment temperature is too high, the crystal grains are coarsened. The heat treatment temperature is preferably 1,200°C.or lower.

Heat treatment time may be suitably a time sufficient for dissolving the precipitate. Most suitable heat treatment time varies depending on the heat treatment temperature but is usually from about 30 minutes to about 2 hours. After the heat treatment, the material is quenched.

### [2.4. Aging Treatment Process]

The aging treatment process is a process of subjecting the material after the solution heat treatment to an aging treatment at a predetermined temperature.

In both cases where aging treatment temperature is too high and too low, an objective precipitate is not precipitated and aging hardening cannot be achieved. The aging treatment temperature is preferably from 600°C to 750°C.

Aging treatment time may be suitably a time sufficient for precipitating a sufficient amount of the precipitate. Most suitable aging treatment time varies depending on the aging treatment temperature but is usually from about 8 hours to about 24 hours.

### [3. Action]

When a predetermined amount of Nb is added to the precipitation hardened Fe-Ni alloy, the γ' phase (Ni₃(Al, Ti, Nb)) and the y" phase (Ni₃Nb) containing Nb as a constituent element are precipitated by the solution heat treatment and the aging treatment.

At this time, when the Nb content is optimized so as to satisfy the formula (2), the precipitation amount of the y" phase is increased. Therefore, as compared with conventional alloys, high strength can be obtained.

On the other hand, as the addition amount of Nb increases, the Laves phase (Fe₂Nb) tends to remain after the solution heat treatment. When a large amount of the Laves phase remains, the Nb amount in the matrix necessary for precipitation hardening decreases. As a result, necessary hardness is not obtained even when the aging treatment is performed.

In contrast, when the Ni content is optimized so as to satisfy the formula (1), the remaining of the Laves phase after the solution heat treatment can be suppressed.

Furthermore, when predetermined amounts of Cr and Mo are added to the precipitation hardened Fe-Ni alloy or predetermined amounts of Cr, Mo and Cu are added to the precipitation hardened Fe-Ni alloy, high corrosion resistance is obtained with maintaining high strength. Particularly, when the contents of Cr, Mo, and Cu are optimized so as to satisfy the formula (3), high corrosion resistance is obtained.

### EXAMPLES

### (Examples 1 to 37, Comparative Examples 1 to 4)

### [1. Preparation of Samples]

After each steel containing various components shown in Tables 1 and 2 was ingoted, each steel was cooled to prepare an ingot. After hot working, the ingot was thermally refined by a solution heat treatment and an aging treatment.

Solution heat treatment temperature was set to 900 to 1,200°C. Also, the aging treatment temperature was set to 600 to 750°C.

**Table 1**

| | Component pomposition (% by mass) | | | | | | | | | | | | | Component balance | | |
|---|---|---|---|---|---|---|---|---|---|---|---|---|---|---|---|---|
| | C | Si | Mn | Ni | Cr | Mo | Al | Ti | Nb | B | Cu | V | Others | Formula (1') | formula (2') | Formula (3') |
| Example 1⁺ | 0.06 | 0.24 | 0.1 | 39.2 | 15.7 | 0.01 | 0.2 | 1.9 | 3.1 | - | | - | | 3.6 | 0.68 | -3.27 |
| Example 2 | 0.05 | 0.41 | 0.5 | 36.9 | 15.4 | 0.03 | 0.2 | 2.3 | 2.7 | 0.0051 | 0.07 | - | | 3.7 | 0.28 | -3.16 |
| Example 3 | 0.06 | 0.46 | 0.3 | 39.8 | 15.8 | 0.13 | 0.5 | 2.1 | 3.2 | 0.0099 | 0.06 | - | | 3.6 | 0.43 | -2.51 |
| Example 4 | 0.04 | 0.35 | 0.3 | 39.8 | 15.4 | 1.54 | 0.3 | 2.4 | 2.7 | 0.0041 | 0.07 | - | | 6.6 | 0.20 | 1.37 |
| Example 5 | 0.04 | 0.35 | 0.3 | 39.8 | 15.4 | 0.52 | 0.3 | 2.4 | 2.7 | 0.0025 | 0.07 | - | | 6.6 | 0.20 | -1.69 |
| Example 6 | 0.05 | 0.39 | 0.6 | 36.8 | 15.0 | 2.40 | 0.2 | 2.2 | 2.7 | 0.0046 | 0.06 | - | | 3.6 | 0.33 | 3.50 |
| Example T | 0.04 | 0.35 | 0.3 | 41.0 | 15.4 | 1.54 | 0.3 | 2.2 | 2.7 | 0.0063 | 0.07 | - | | 7.8 | 0.28 | 1.37 |
| Example 8 | 0.04 | 0.35 | 0.3 | 38.9 | 15.4 | 0.53 | 0.3 | 2.2 | 2.7 | 0.0006 | 0.52 | - | | 5.7 | 0.28 | 0.59 |
| Example 9 | 0.04 | 0.35 | 0.3 | 38.9 | 15.4 | 0.52 | 0.3 | 2.2 | 2.7 | 0.0051 | 0.07 | 0.5 | | 5.7 | 0.28 | -1.69 |
| Example 10 | 0.04 | 0.35 | 0.3 | 38.9 | 17.8 | 0.52 | 0.3 | 2.2 | 2.7 | 0.0099 | 0.07 | - | | 5.7 | 0.28 | 0.71 |
| Example 11 | 0.04 | 0.35 | 0.3 | 38.9 | 19.5 | 0.52 | 0.3 | 2.2 | 2.7 | 0.0041 | 0.07 | - | | 5.7 | 0.28 | 2.41 |
| Example 12 | 0.04 | 0.35 | 0.3 | 36.4 | 15.4 | 0.52 | 0.3 | 2.2 | 2.7 | 0.0025 | 0.07 | - | | 3.2 | 0.28 | -1.69 |
| Example 13 | 0.04 | 0.35 | 0.3 | 38.9 | 15.4 | 0.52 | 0.3 | 2.2 | 2.2 | 0.0046 | 0.07 | - | | 8.7 | 0.08 | -1.69 |
| Example 14 | 0.04 | 0.35 | 0.3 | 38.9 | 15.4 | 0.52 | 0.3 | 2.2 | 3.4 | 0.0063 | 0.07 | - | | 1.5 | 0.56 | -1.69 |
| Example 15 | 0.04 | 0.35 | 0.3 | 38.9 | 15.4 | 0.52 | 0.9 | 2.2 | 2.7 | 0.0006 | 0.07 | - | | 5.7 | 0.07 | -1.69 |
| Example 16 | 0.04 | 0.35 | 0.3 | 38.9 | 15.4 | 0.52 | 0.3 | 1.3 | 2.7 | 0.0051 | 0.07 | - | | 5.7 | 0.89 | -1.69 |
| Example 17 | 0.04 | 0.35 | 0.3 | 38.9 | 15.4 | 0.52 | 0.3 | 2.4 | 2.7 | 0.0099 | 0.07 | - | | 5.7 | 0.20 | -1.69 |
| Example 18 | 0.04 | 0.82 | 0.3 | 38.9 | 15.4 | 0.52 | 0.3 | 2.2 | 2.7 | 0.0041 | 0.07 | - | Zr:0.05 | 5.7 | 0.28 | -1.69 |
| Example 19 | 0.04 | 0.35 | 0.3 | 38.9 | 15.4 | 0.52 | 0.3 | 2.2 | 2.7 | 0.0025 | 0.07 | - | Ta:0.15 | 5.7 | 0.28 | -1.69 |
| Example 20 | 0.04 | 0.35 | 0.3 | 38.9 | 15.4 | 0.52 | 0.3 | 2.2 | 2.7 | 0.0046 | 0.07 | - | W:0.32 | 5.7 | 0.28 | -1.69 |
| Example 21 | 0.04 | 0.35 | 0.3 | 38.9 | 15.4 | 0.52 | 0.3 | 2.2 | 2.7 | 0.0063 | 0.07 | - | Hf:0.21 | 5.7 | 0.28 | -1.69 |

| | | | | | | | | | | | | | | | | |
|---|---|---|---|---|---|---|---|---|---|---|---|---|---|---|---|---|
| * Formula (1') = Ni-(6×Nb+17), Formula (2')=Nb/(Ti+Al)-0.8, Formula (3') = Cr+3Mo+5Cu-19 ⁺ not forming part of the invention. | | | | | | | | | | | | | | | | |

**Table 2**

| | Component composition (% by mass) | | | | | | | | | | | | | Component balance | | |
|---|---|---|---|---|---|---|---|---|---|---|---|---|---|---|---|---|
| | C | Si | Mn | Ni | Cr | Mo | Al | Ti | Nb | B | Cu | V | Others | Formula (1') | Formula (2') | Formula (3') |
| Example 22 | 0.04 | 0.35 | 0.3 | 38.9 | 15.4 | 0.52 | 0.3 | 2.2 | 2.7 | 0.0006 | 0.07 | - | Mg:0.02 | 5.7 | 0.28 | -1.69 |
| Example 23 | 0.04 | 0.35 | 0.3 | 38.9 | 15.4 | 0.52 | 0.3 | 2.2 | 2.7 | 0.0046 | 0.07 | - | REM:0.03 | 5.7 | 0.28 | -1.69 |
| Example 24 | 0.04 | 0.35 | 0.3 | 38.9 | 15.4 | 0.52 | 0.3 | 2.2 | 2.7 | 0.0063 | 0.07 | - | Ca:0.004 | 5.7 | 0.28 | -1.69 |
| Example 25 | 0.04 | 0.35 | 0.3 | 38.9 | 15.4 | 1.62 | 0.3 | 2.2 | 2.7 | 0.0006 | 0.61 | - | | 5.7 | 0.28 | 4.31 |
| Example 26 | 0.04 | 0.35 | 0.3 | 38.0 | 15.7 | 0.01 | 0.2 | 2.2 | 2.7 | 0.0011 | | - | | 4.8 | 0.33 | -3.27 |
| Example 27 | 0.04 | 0.35 | 0.3 | 38.0 | 15.4 | 0.03 | 0.3 | 2.4 | 2.5 | 0.0023 | | - | | 6.0 | 0.13 | -3.51 |
| Example 28 | 0.04 | 0.35 | 0.6 | 38.0 | 15.8 | 0.13 | 0.2 | 2.2 | 2.7 | 0.0005 | 0.36 | - | | 4.8 | 0.33 | -1.01 |
| Example 29 | 0.04 | 0.35 | 0.5 | 38.0 | 15.4 | 1.54 | 0.3 | 2.2 | 2.5 | 0.0042 | 0.09 | - | | 6.0 | 0:20 | 1.47 |
| Example 30 | 0.04 | 0.24 | 0.4 | 38.0 | 15.4 | 0.52 | 0.2 | 2.2 | 2.7 | 0.0051 | | - | | 4.8 | 0.33 | -2.04 |
| Example 31 | 0.04 | 0.24 | 0.5 | 38.0 | 17.8 | 0.53 | 0.3 | 2.2 | 2.5 | 0.0048 | | - | | 6.0 | 0.20 | 0.39 |
| Example 32 | 0.05 | 0.24 | 0.6 | 38.0 | 19.5 | 0.52 | 0.2 | 1.5 | 2.7 | 0.0045 | 0.43 | - | | 4.8 | 0.79 | 4.21 |
| Example 33 | 0.05 | 0.46 | 0.3 | 38.0 | 15.4 | 0.52 | 0.3 | 2.2 | 2.5 | 0.0029 | 0.05 | - | | 6.0 | 0.20 | -1.79 |
| Example 34 | 0.05 | 0.46 | 0.3 | 38.0 | 15.4 | 0.51 | 0.2 | 2.2 | 2.7 | 0.0055 | | 0.3 | | 4.8 | 0.33 | -2.07 |
| Example 35 | 0.05 | 0.46 | 0.3 | 38.0 | 15.6 | 0.51 | 0.3 | 2.2 | 2.5 | 0.0061 | | 0.4 | | 6.0 | 0.20 | -1.87 |
| Example 36 | 0.05 | 0.46 | 0.3 | 38.0 | 15.8 | 0.52 | 0.2 | 2.2 | 2.7 | 0.0053 | 0.57 | 0.4 | | 4.8 | 0.33 | 1.21 |
| Example 37 | 0.05 | 0.46 | 0.3 | 38.0 | 15.9 | 0.52 | 0.3 | 2.2 | 2.5 | 0.0048 | | 0.5 | | 6.0 | 0.20 | -1.54 |
| Comparative Example 1 | 0.03 | 0.31 | 0.2 | 25.1 | 15.0 | 1.1 | 0.2 | 2.2 | - | - | | 0.3 | | | | |
| Comparative Example 2 | 0.04 | 0.35 | 0.3 | 33.8 | 15.4 | 0.52 | 0.3 | 2.2 | 2.7 | 0.0041 | 0.07 | - | | 0.6 | 0.28 | -1.69 |
| Comparative Example 3 | 0.04 | 0.35 | 0.3 | 36.3 | 15.4 | 0.52 | 0.5 | 2.2 | 2.0 | 0.0041 | 0.07 | - | | 7.3 | -0.06 | -1.69 |
| Comparative Example 4 | 0.04 | 0.35 | 0.3 | 36.3 | 15.4 | 0.52 | 0.3 | 2.2 | 3.4 | 0.0041 | 0.07 | - | | -1.1 | 0.56 | -1.69 |

| | | | | | | | | | | | | | | | | |
|---|---|---|---|---|---|---|---|---|---|---|---|---|---|---|---|---|
| * Formula (1') = Ni-(6×Nb+17), Formula (27) = Nb/(Ti+Al)-0.8, Formula (3') = Cr+3Mo+5Cu-19 | | | | | | | | | | | | | | | | |

### [2. Test Methods]

### [2.1. Tensile Test]

From each material after the aging treatment, a JIS No. 4 test piece was cut out. A tensile test was performed at room temperature (20°C) to evaluate tensile strength and 0.2% offset yield strength.

### [2.2. Corrosion Resistance Test]

Evaluation of the corrosion resistance was performed on a corrosion rate at the time of immersion for 6 h in 10% hydrochloric acid at 80°C. The case where the corrosion rate was 100 g/m²/h or less was designated as "A", the case where the rate was more than 100 g/m²/h and 200 g/m²/h or less was designated as "B", and the case where the rate was more than 200 g/m²/h was designated as "C".

### [2.3. Carbide Area Percentage]

For quantitative analysis of a carbide, area percentage was measured at 30 visual fields on a microstructure photograph with a magnification of 400 times (1 visual field: 0.034 mm²) using an image-analyzing software.

### [3. Results]

Table 3 shows results. From Table 3, the following are realized.
(1) In Comparative Example 1 (corresponding to A286 alloy), the tensile strength and the 0.2% offset yield strength are low. This is because Nb is not added and the y" phase is not precipitated. Also, in Comparative Example 1, the corrosion resistance is low. This is because the Ni amount is small.
(2) In Comparative Example 2, the 0.2% offset yield strength is slightly low. This is because the Ni content is small and hence a sufficient amount of the y" phase is not obtained. Also, in Comparative Example 2, the corrosion resistance is low. This is because the Ni amount is small.
(3) In Comparative Example 3, the 0.2% offset yield strength is slightly low. This is because a sufficient amount of the γ" phase is not obtained owing to a low value of Nb/(Ti+Al)-0.8.
(4) In Comparative Example 4, the 0.2% offset yield strength is slightly low. This is because a coarse Laves phase remains owing to a low value of Ni-(6×Nb+17) and, as a result, the Nb amount in the matrix is decreased and hence the precipitation amounts of the γ' phase and the γ" phase at the time of the aging treatment are decreased.
(6) In all of Examples 1 to 37, the 0.2% offset yield strength is more than 850 MPa and good corrosion resistance is exhibited.
(7) Among Examples, the materials satisfying the formula (3) particularly exhibit high corrosion resistance.

**Table 3**

| | Tensile strength (MPa) | 0.2% offset yield strength (MPa) | Corrosion resistance | Carbide area percentage (%) |
|---|---|---|---|---|
| Example 1⁺ | 1168 | 972 | B | 0.73 |
| Example 2 | 1160 | 929 | B | 0.68 |
| Example 3 | 1191 | 990 | B | 0.74 |
| Example 4 | 1153 | 961 | A | 0.51 |
| Example 5 | 1196 | 946 | B | 0.53 |
| Example 6 | 1137 | 894 | A | 0.59 |
| Example 7 | 1163 | 972 | A | 0.48 |
| Example 8 | 1160 | 969 | A | 0.49 |
| Example 9 | 1193 | 945 | B | 0.54 |
| Example 10 | 1162 | 931 | A | 0.50 |
| Example 11 | 1142 | 924 | A | 0.55 |
| Example 12 | 1132 | 866 | B | 0.52 |
| Example 13 | 1175 | 888 | B | 0.47 |
| Example 14 | 1227 | 997 | B | 0.61 |
| Example 15 | 1197 | 948 | B | 0.45 |
| Example 16 | 1173 | 857 | B | 0.41 |
| Example 17 | 1206 | 937 | B | 0.60 |
| Example 18 | 1198 | 948 | B | 0.52 |
| Example 19 | 1187 | 936 | B | 0.54 |
| Example 20 | 1203 | 952 | B | 0.53 |
| Example 21 | 1193 | 942 | B | 0.58 |
| Example 22 | 1186 | 941 | B | 0.51 |
| Example 23 | 1188 | 937 | B | 0.54 |
| Example 24 | 1192 | 945 | B | 0.49 |
| Example 25 | 1137 | 894 | A | 0.55 |
| Example 26 | 1152 | 963 | B | 0.53 |
| Example 27 | 1163 | 984 | B | 0.58 |
| Example 28 | 1155 | 966 | A | 0.42 |
| Example 29 | 1148 | 957 | B | 0.47 |
| Example 30 | 1166 | 987 | B | 0.54 |
| Example 31 | 1152 | 964 | A | 0.61 |
| Example 32 | 1141 | 887 | A | 0.68 |
| Example 33 | 1159 | 989 | B | 0.72 |
| Example 34 | 1164 | 977 | B | 0.71 |
| Example 35 | 1161 | 983 | B | 0.66 |
| Example 36 | 1142 | 850 | A | 0.65 |
| Example 37 | 1172 | 887 | B | 0.69 |
| Comparative Example 1 | 1052 | 651 | C | 0.35 |
| Comparative Example 2 | 1166 | 850 | C | 0.53 |
| Comparative Example 3 | 1004 | 843 | C | 0.52 |
| Comparative Example 4 | 1018 | 827 | C | 0.55 |

| | | | | |
|---|---|---|---|---|
| ⁺ not forming part of the invention | | | | |

Fig. 1 shows optical microscopic photographs of materials after solution heat treatment obtained in Example 5 and Comparative Example 4. From Fig. 1, it is realized that the Laves phase is observed besides the carbide in Comparative Example 4.

While the mode for carrying out the present invention has been described in detail above, the present invention is not limited to these embodiments, any various changes and modifications can be made therein without departing from the present invention as set out in the appended claims.

### INDUSTRIAL APPLICABILITY

The precipitation hardened Fe-Ni alloy according to the invention can be used as members for excavation, automobile engine parts, thermal power generation plant members, and the like.

## Claims

1. A precipitation hardened Fe-Ni alloy having the following constitutions:
the precipitation hardened Fe-Ni alloy consisting of:
from 0.01 to 0.08% by mass of C,
from 0.02 to 1.0% by mass of Si,
not more than 1.0% by mass of Mn,
from 36.0 to 41.0% by mass of Ni,
14.0 or more and less than 20.0% by mass of Cr,
from 0.01 to 3.0% by mass of Mo,
from 0.1 to 1.0% by mass of Al,
from 1.0 to 2.5% by mass of Ti,
from 2.0 to 3.5% by mass of Nb, and
from 0.0005 to 0.01% by mass of B,
optionally comprising:
0.05 to 1.0% by mass of Cu,
0.05 to 1.0% by mass of V,
0.001 to 0.50% by mass of Zr, Ta, W, Hf, Mg, and REM in total, and
from 0.0005 to 0.01% by mass of Ca,
with the balance being Fe and unavoidable impurities;
the precipitation hardened Fe-Ni alloy satisfying the following formulae (1) and (2): $Ni \geq 6 \times Nb + 17$ $Nb / \left(Ti+Al\right) \geq 0.8$

2. The precipitation hardened Fe-Ni alloy according to claim 1, comprising from 0.0010 to 0.008% by mass of B.

3. The precipitation hardened Fe-Ni alloy according to claim 1 or 2, comprising from 0.10 to 1.0% by mass of Cu.

4. The precipitation hardened Fe-Ni alloy according to any one of claims 1 to 3, wherein the 0.2% offset yield strength at room temperature is 850 MPa or more.

5. The precipitation hardened Fe-Ni alloy according to claim 4, wherein the 0.2% offset yield strength at room temperature is 900 MPa or more.

6. The precipitation hardened Fe-Ni alloy according to any one of claims 1 to 5, further satisfying the following formula (3): $Cr + 3 ⁢ Mo + 5 ⁢ Cu \geq 19$

## Patentansprüche

1. Ausscheidungsgehärtete Fe-Ni Legierung mit folgender Zusammensetzung:
die ausscheidungsgehärtete Fe-Ni Legierung bestehend aus:
von 0,01 bis 0,08 Massenprozent C,
von 0,02 bis 1,0 Massenprozent Si,
nicht mehr als 1,0 Massenprozent Mn,
von 36,0 bis 41,0 Massenprozent Ni,
14,0 oder mehr und weniger als 20,0 Massenprozent Cr,
von 0,01 bis 3,0 Massenprozent Mo,
von 0,1 bis 1,0 Massenprozent Al,
von 1,0 bis 2,5 Massenprozent Ti,
von 2,0 bis 3,5 Massenprozent Nb, und
von 0,0005 bis 0,01 Massenprozent B,
optional aufweisend:
0,05 bis 1,0 Massenprozent Cu,
0,05 bis 1,0 Massenprozent V,
insgesamt 0,001 bis 0,50 Massenprozent Zr, Ta, W, Hf, Mg, und REM, und
von 0,0005 bis 0,01 Massenprozent Ca,
wobei der Rest Fe und unvermeidbare Verunreinigungen ist;
wobei die ausscheidungsgehärtete Fe-Ni Legierung die folgenden Bedingungen (1) und (2) erfüllt: $Ni \geq 6 \times Nb + 17$ $Nb / \left(Ti+Al\right) \geq 0 , 8$

2. Ausscheidungsgehärtete Fe-Ni Legierung nach Anspruch 1, aufweisend von 0,0010 bis 0,008 Massenprozent B.

3. Ausscheidungsgehärtete Fe-Ni Legierung nach Anspruch 1 oder 2, aufweisend von 0,10 bis 1,0 Massenprozent Cu.

4. Ausscheidungsgehärtete Fe-Ni Legierung nach einem der Ansprüche 1 bis 3, wobei die 0,2% Dehngrenze bei Raumtemperatur 850 MPa oder mehr beträgt.

5. Ausscheidungsgehärtete Fe-Ni Legierung nach Anspruch 4, wobei die 0,2 % Dehngrenze bei Raumtemperatur 900 MPa oder mehr beträgt.

6. Ausscheidungsgehärtete Fe-Ni Legierung nach einem der Ansprüche 1 bis 5, weiter erfüllend die folgende Bedingung (3): $Cr + 3 ⁢ Mo + 5 ⁢ Cu \geq 19$

## Revendications

1. Alliage Fe-Ni durci par précipitation ayant les constitutions suivantes :
l'alliage Fe-Ni durci par précipitation consistant en :
de 0,01 à 0,08 % en masse de C,
de 0,02 à 1,0 % en masse de Si,
pas plus de 1,0 % en masse de Mn,
de 36,0 à 41,0 % en masse de Ni,
14,0 ou plus et moins de 20,0 % en masse de Cr,
de 0,01 à 3,0 % en masse de Mo,
de 0,1 à 1,0 % en masse d'Al,
de 1,0 à 2,5 % en masse de Ti,
de 2,0 à 3,5 % en masse de Nb, et
de 0,0005 à 0,01 % en masse de B,
comprenant éventuellement :
0,05 à 1,0 % en masse de Cu,
0,05 à 1,0 % en masse de V,
0,001 à 0,50 % en masse de Zr, Ta, W, Hf, Mg et REM au total, et
de 0,0005 à 0,01 % en masse de Ca,
le reste étant Fe et des impuretés inévitables,
l'alliage Fe-Ni durci par précipitation satisfaisant les formules (1) et (2) suivantes : $Ni \geq 6 \times Nb + 17$ $Nb / \left(Ti+Al\right) \geq 0 , 8$

2. Alliage Fe-Ni durci par précipitation selon la revendication 1, comprenant de 0,0010 à 0,008 % en masse de B.

3. Alliage Fe-Ni durci par précipitation selon la revendication 1 ou 2, comprenant de 0,10 à 1,0 % en masse de Cu.

4. Alliage Fe-Ni durci par précipitation selon l'une quelconque des revendications 1 à 3, dans lequel la limite d'élasticité à une déformation de 0,2 % à température ambiante est de 850 MPa ou plus.

5. Alliage Fe-Ni durci par précipitation selon la revendication 4, dans lequel la limite d'élasticité à une déformation de 0,2 % à température ambiante est de 900 MPa ou plus.

6. Alliage Fe-Ni durci par précipitation selon l'une quelconque des revendications 1 à 5, satisfaisant en outre la formule (3) suivante : $Cr + 3 ⁢ Mo + 5 ⁢ Cu \geq 19$
